

Oct. 15, 1963

H. KURZKE, ETAL

3,107,140

PROCESS FOR THE MANUFACTURE OF FIBERS AND FILAMENTS OF  
LINEAR POLYESTERS HAVING IMPROVED PROPERTIES

Filed Aug. 8, 1961

Fig. 1.  
TREATMENT OF A FIBER CABLE ACCORDING TO THE  
PRESENT INVENTION (NUMERICAL VALUES ACCORDING TO EXAMPLE 4)



Fig. 2.

CONTACT HEATING DEVICE WITH LAYER OF FIBERGLASS  
TISSUE ACCORDING TO THE PRESENT INVENTION

HEATED BARRIER SHEET



INVENTORS

HERBERT KURZKE  
HELMUT SATTLER  
EDMUND STIX

BY *Connolly and Flory* ATTORNEYS

3,107,140

PROCESS FOR THE MANUFACTURE OF FIBERS  
AND FILAMENTS OF LINEAR POLYESTERS  
HAVING IMPROVED PROPERTIES

Herbert Kurzke, Helmut Sattler, and Edmund Stix, all of Bobingen, near Augsburg, Germany, assignors to Farbwerke Hoechst Aktiengesellschaft vormals Meister Lucius & Brüning, Frankfurt am Main, Germany, a corporation of Germany

Filed Aug. 8, 1961, Ser. No. 129,979

Claims priority, application Germany Aug. 13, 1960  
8 Claims. (Cl. 18—43)

The present invention relates to the manufacture of fibers or filaments of linear aromatic polyesters and more particularly it relates to the manufacture of fibers and filaments of linear aromatic polyesters having improved properties.

The present invention provides a process for making fibers and filaments of linear aromatic polyesters which have a good dyeability. Moreover, the present invention provides a process for making fibers and filaments of linear aromatic polyesters having a low tendency to pilling.

Fibers or filaments of linear polyesters, especially of polyethylene terephthalate, possess a number of special advantages but, in addition thereto, they have the disadvantage that they are difficult to dye. Hitherto, the fibers or filaments have mostly been dyed with the use of so-called carriers and with the application of especially high temperature. These dyeing methods require special care and need expensive apparatus, particularly when piece goods are to be dyed.

It has now been found that fibers and filaments can be produced in simple manner and in continuous operation from linear polyesters, and especially from polyethylene terephthalate, which possess a considerably improved dyeability.

The present invention is concerned with a process for the manufacture of fibers and filaments of linear polyesters having an improved dyeability. A spinning cable or filament of linear polyesters, especially of polyethylene terephthalate, or of a mixed polyester, is stretched under cold and/or heated conditions in one or several stages to a multiple of its original length, then allowed to shrink by 8 to 40% at a temperature above 190° C., preferably at 220° C., and subsequently stretched a second time under cold and/or heated conditions by at least 3% and at most up to the breaking limit of the cable or filament.

It is suitable to use a spinning cable of polyethylene terephthalate having for example a total titer of several hundred thousand denier and to stretch said cable in steam, hot water or hot air to a multiple of its original length with the aid of known roller units. The degree of stretching can vary within wide limits, depending on the intended application or the desired textile properties of the fiber. Instead of carrying out the stretching in steam or hot air, it can be realized in exceptional cases without the action of heat in the cold.

The shrinking process, which is carried out after the stretching, is preferably performed with the aid of hot air or by conducting the cable over a heated surface. The lower temperature limit shall not be lower than 190° C. The temperature given is, as in the stretching, the temperature of the heat transferring medium. The upper temperature limit in the shrinking process is at most 250° C. for fibers and up to 310° C. for filaments that are treated for a short period of time.

The admissible shrinkage in the shrinking process is 8-40%, depending on the properties of the material used for making the fibers (for example the specific viscosity of the polyester) or the chosen stretching conditions.

When a low viscous starting material is used and with a stretching ratio of 1:3.8, the shrinkage is only 10%, while in the case of a highly viscous material and with a stretching ratio of 1:4.2 the fiber can be allowed to shrink by 30%.

The cable which has been allowed to shrink in this manner has an especially improved dyeability. Moreover, the fibers obtained practically do not undergo further shrinkage in boiling water or in hot air, provided that the air temperature is not higher than the temperature in the shrinking process. If the fibers were thermally treated at the indicated temperature without being allowed to shrink, their dyeability could be immaterially improved only.

Finally, the cable is again stretched under cold and/or heated conditions. The stretching degree ranges from 3% up to the breaking limit of the cable. By the selection of the stretching ratio and the kind of stretching, with steam, under hot or cold conditions, fibers or filaments can be obtained having the desired shrinking values for a definite application. The shrinking values of the fibers or filaments on boiling in water can range from 0 to 20% and on heating in hot air of 200° C. they can range from 2 to 30%.

It is surprising that by the after-stretching process (second stretching) the improved dyeability obtained by the shrinking is not impaired. Thus it is possible to produce by the process of the invention fibers and filaments of polyethylene terephthalate having an especially good dyeability, good physical properties, an adjustable shrinkage in boiling water and an adjustable thermo-shrinkage.

When fibers or filaments having different shrinking properties are worked up together very voluminous yarns can be obtained (bulk yarns).

For the manufacture of fibers and filaments of linear polyesters, especially of polyethylene terephthalate, there are generally used polymers having an average molecular weight corresponding to a specific viscosity of 0.78-0.84. The specific viscosity is the ratio, reduced by 1, of the viscosity of the solution of the polyester in a mixture of 60 parts of phenol and 40 parts of tetrachloroethane to the viscosity of the solvent, the viscosities being determined by the time a fixed volume needs to flow through an Ubbelohde viscometer.

Recently, fibers and filaments having favorable properties, for example a low tendency to pilling, are made from polyethylene terephthalate of low medium molecular weight. However, fibers of this kind are more difficult to dye by various dyestuffs than fibers of polyethylene terephthalate having the usual medium molecular weight.

Moreover, it has been found that little pilling occurs and well dyeable fibers and filaments can be made by the process of the invention when the fibers or filaments are produced from polyethylene terephthalate having a specific viscosity below 0.5. It is remarkable that the fibers and filaments of polyethylene terephthalate having a specific viscosity below 0.5, which have been produced by the process of the invention, can be dyed more easily than products that have been made in the same manner from polyethylene terephthalate having a specific viscosity of 0.78-0.84. This could not be expected since the dyeability of fibers and filaments produced by the usual manufacturing process diminishes with a series of dyestuffs as the medium molecular weight, i.e. the specific viscosity, decreases. Thus it is of advantage, not only on account of the improved textile properties but also in view of the still further improved dyeability, to use in the manufacture of the fibers and filaments used in the present process polyethylene terephthalate having

an especially low medium molecular weight, corresponding to a specific viscosity below 0.5.

When fibers and filaments from polyethylene terephthalate having an especially low medium molecular weight, are spun and worked up, the final products obtained may have defects, for example agglutinating individual fibers and drop-like knots, which impair the further working up of the fibers and filaments into textile materials.

These defects result from the fact that the individual filaments leaving the spinning nozzle of polyethylene terephthalate having a low medium molecular weight are not so tough as filaments of normal polyethylene terephthalate leaving the nozzle and thus agglutinate more readily with one another. A preferred embodiment of the process of the invention consists in spinning polyethylene terephthalate having a very low medium molecular weight, corresponding to a specific viscosity below 0.5 in admixture with a small proportion of up to 20%, and preferably 10%, of polyethylene terephthalate having a normal medium molecular weight and a specific viscosity in the range from 0.78 to 0.84, and treating the fibers and filaments obtained as described above. By this mode of operation the textile properties of the fibers and filaments are not modified and their dyeability is not impaired, but the spinning process is facilitated and fewer agglutinations and other defects can be observed.

Polyethylene terephthalate having a very low medium molecular weight is often obtained in the polycondensation with a non uniform distribution of the molecular weight, so that when spinning from the melt the individual filaments leaving the spinning nozzle have a non uniform toughness in themselves and against one another whereby filaments of varying thickness as well as knots may be formed. This difficulty can be overcome by melting polyethylene terephthalate having a specific viscosity below 0.5, prior to spinning the fibers from the melt, in a known device with the exclusion of air, extruding it into a wire some millimeters thick, cutting the wire into chips and feeding the chips to the spinning unit. By this pretreatment the polyethylene terephthalate is homogenized and intimately mixed. Either mode of operation, namely the admixture of a small proportion of polyethylene terephthalate having a normal medium molecular weight or the homogenization of the polyethylene terephthalate by melting it prior to the spinning process overcomes the above disadvantages when applied individually or jointly. It is especially advantageous to mix polyethylene terephthalate having a specific viscosity below 0.5 with a small proportion of up to 20%, and preferably 10%, of polyethylene terephthalate having a normal medium molecular weight, i.e. a specific viscosity in the range from 0.78 to 0.84, to melt the mixture obtained in a known device with the exclusion of air, to form a wire having a thickness of several millimeters by extrusion, to cut the wire into chips and to feed the chips to the actual spinning device for being spun from the melt. By this pretreatment the mixture of the two polyethylene terephthalates is homogenized and the favorable action of the proportion of polyethylene terephthalate having a normal medium molecular weight is improved. By this pretreatment the number of spinning defects in the final product is further reduced.

For uniformly heating the cable of fibers or filaments it is passed over a heated surface while being in contact therewith. If the temperature of the surface is too high, the fibers and filaments may adhere to the heated surface. This is favored by the fact that the material is under a slight tension on account of the shrinkage. The adhering fibers soil the heated surface of the heating device and above all, they disturb the further working up of the fibers. In general it is, therefore, not recommended to heat the surface at a temperature above 220° C.

However, the temperature of the heated surface, the temperature of the fibrous material and the degree of

shrinkage can be surprisingly increased when the surface over which the cable of fibers or filaments is passed after the first stretching to undergo shrinkage is coated with a thin, smooth layer of a material having poor heat-conducting properties. A coating of this kind prevents the fibers or filaments from adhering to the surface of contact and, furthermore, in such a thin, smooth layer having poor heat-conducting properties a temperature gradient is formed which results in a more uniform heating of the cable of fibers than in case the cable contacts directly the metallic heating surface. By the process of the invention the fiber cable is heated to a higher temperature and more uniformly so that it can then be dyed more intensely and more uniformly and is substantially free from agglutinations.

As layers having poor heat-conducting properties there can be used narrow and wide-meshed fabrics of temperature resisting materials, and heatproof closed or perforated films.

According to a preferred embodiment of the process of the invention the heated surface, over which the filaments or cable of fibers are passed, is coated with a fabric of endless glass filaments or yarns of glass fibers. This fabric forms a thin and smooth layer having poor heat conducting properties that withstands the temperatures applied and the friction of the fiber cable.

In order to avoid losses of heat and to maintain constant the desired temperature, it is often of advantage to arrange a heated plate above the heated surface, which plate, however, does not come into contact with the fiber cable.

Moreover, it is of advantage carefully to dry the fiber cable before it enters the heated shrinking zone. Thus heating energy is saved in the shrinking zone and the fiber cable really picks up the temperature of the heated surface covered with a fabric of endless glass filaments or yarns of glass fibers. Furthermore, the danger of the hydrolytic decomposition of the polyester by water at the high temperature of the heating device is reduced. The cable can be dried according to common methods, for example by passing it over a surface heated at a temperature above 100° C. or by heating internally the conveying rollers of the cable.

The following examples serve to illustrate the invention but they are not intended to limit it thereto. In the examples the medium molecular weight or the polymerization degree of the polyethylene terephthalate used is defined by the specific viscosity  $\eta_{sp}$ , determined with a 1% solution of the polymer in a mixture of 60 parts of phenol and 40 parts of tetrachloroethane in an Ubbelohde viscometer. The specific viscosity is the ratio minus 1 of the viscosity of the solution of the polymer to the viscosity of the solvent.

For determining the dyestuff receptivity 20 grams of the fiber sample were boiled for one hour in 1 liter of a bath containing 3%, calculated on the weight of the sample, of the dyestuff obtained by brominating 1,5-diamino-4,8-dihydroxy-anthraquinone. The residual dyestuff in the bath was determined by colorimetric means and the dyestuff receptivity of the sample was calculated in percent of the dyestuff used.

The process of the invention is better shown in FIGURES 1 and 2 of the drawing. The temperatures, rotational speed of the rolls and other values set forth on the drawing are taken from Example 4 of the specification. As shown by the legends in FIGURE 1, the unstretched filament cable is first stretched with steam between rolls wherein the second set of rolls rotates at a faster rate of speed than the first set. The cable is then shrunk under heated conditions with the use of the heat barrier assembly shown better in FIGURE 2. The set of rolls drawing the cable through the shrinking unit rotates at a slower rate of speed than the set feeding the cable through the shrinking unit. The cable is then stretched a second time under heated conditions with the use of the heat barrier unit of FIGURE 2. However, in this stage of the second

stretching, the layer of Fiberglas tissue can be omitted if desired. The final set of rolls drawing the cable to the second stretching station is rotated at a faster r.p.m. than the set of rolls feeding the cable to the second stretching station.

The heat barrier unit of FIGURE 2 is self-explanatory from an examination of the legends of the figure. Here, the cable being treated passes in contact with a Fiberglas layer which overlies a heating block. A heat barrier sheet is positioned in spaced-apart relationship above the Fiberglas sheet and the assumed path of the cable.

### EXAMPLE 1

A spinning thread of 180 denier composed of 25 individual filaments of polyethylene terephthalate having a specific viscosity  $\eta_{sp}$  of 0.84 was continuously stretched at 110° C. as usual to 4 times its original length with contact heating, and wound up on a bobbin. The thread was then passed, at a rate of 30 meters per minute, into a heating flue having a length of 20 cm. and a temperature of 250° C., in which it was allowed to shrink by 30% calculated on the feed rate, by the following conveying means. The thread was then stretched continuously in the cold to its original length. Prior to the shrinkage and in the final state the thread had the following textile properties:

|                      | Stretched thread prior to shrinkage | Final State   |
|----------------------|-------------------------------------|---------------|
| Titer                | 45.7 denier                         | 44.9 denier.  |
| Tensile strength     | 3.9 g/denier                        | 4.0 g/denier. |
| Elongation at break  | 19.7%                               | 20.3%         |
| Shrinkage at 200° C. | 20.4%                               | 23.5%         |
| Dyestuff receptivity | 19.0%                               | 43.5%         |

### EXAMPLE 2

A spinning cable having a total titer of 370,000 denier and a spinning titer (prior to stretching) of the individual filaments of 11.7 denier of polyethylene terephthalate having a specific viscosity  $\eta_{sp}$  of 0.80 was stretched in steam, then allowed to shrink continuously while being heated with contact heating and again stretched while heated with contact heating. The cable was subsequently treated with a scrooping agent, crimped and cut. The conveying speeds of the individual stages and the textile properties of the final product are listed in the following Table 1.

### EXAMPLE 3

A spinning cable was produced from the polyethylene terephthalate defined in Example 2 having a total titer of 340,000 denier and a spinning titer of the individual filaments of 5.1 denier. The cable was treated as described in Example 2. The data and the textile properties of the final product are given in the following Table 1.

### EXAMPLE 4

A spinning cable having a total titer of 370,000 denier and a spinning titer of the individual filaments of 11.7 denier was made from polyethylene terephthalate having a specific viscosity  $\eta_{sp}$  of 0.545 and the cable was treated as described in Example 2. The data and textile properties of the cable are listed in the following Table 1.

In the following table the data and textile properties of the cables are compared with the data and properties of a cable as defined in Example 2 which was stretched but not allowed to shrink.

6  
Table 1

|    | Example No.                          | 2       | 3       | 4       | Comparison |
|----|--------------------------------------|---------|---------|---------|------------|
| 5  | $\eta_{sp}$ of polymer               | 0.80    | 0.80    | 0.545   | 0.80       |
|    | Total titer of cable, denier         | 370,000 | 340,000 | 370,000 | 370,000    |
|    | Titer of individual filament, denier | 11.7    | 5.1     | 11.7    | 11.7       |
|    | Conveying speed in m/minute:         |         |         |         |            |
| 10 | Prior to stretching                  | 10.1    | 10.5    | 10.5    | 10.1       |
|    | After stretching                     | 45.3    | 43.6    | 43.5    | 45.3       |
|    | After shrinkage                      | 34.7    | 33.6    | 36.4    | -----      |
|    | After second stretching              | 37.8    | 38.4    | 43.3    | -----      |
|    | Temperature, °C.:                    |         |         |         |            |
|    | During shrinkage                     | 240     | 240     | 240     | -----      |
|    | During second stretching             | 120     | 150     | 150     | -----      |
| 15 | Individual titer, denier             | 3.4     | 1.6     | 3.1     | 3.0        |
|    | Tensile strength g/denier            | 4.7     | 5.2     | 3.6     | 5.0        |
|    | Elongation at break, percent         | 56      | 33.5    | 44.3    | 42.6       |
|    | Shrinkage at 200° C., percent        | 4.1     | 7.3     | 8.7     | 11.3       |
|    | Dyestuff receptivity, percent        | 41.7    | 39.7    | 63.8    | 16.7       |

The above Table 1 shows that the process of the invention permits the manufacture of filaments and fibers of polyethylene terephthalate having a considerably improved dyestuff receptivity, the other textile values remaining the same.

### EXAMPLE 5

Polyethylene terephthalate having a specific viscosity  $\eta_{sp}$  of 0.46 was spun from the melt and a spinning cable was formed having a total titer of 600,000 denier and a spinning titer (unstretched titer) of the individual filaments of 11.7 denier. The cable was stretched as described in Example 2, then continuously allowed to shrink while being heated by contact heating, and subsequently stretched again while heated. The cable was then treated with a scrooping agent, crimped and cut. The conveying speeds in the individual stages and the textile properties of the final product are listed in the following Table 2.

### EXAMPLE 6

A mixture of 90 parts of polyethylene terephthalate having a specific viscosity  $\eta_{sp}$  of 0.46 and 10 parts of polyethylene terephthalate having a specific viscosity  $\eta_{sp}$  of 0.82 was spun from the melt and a spinning cable was formed having a total titer of 150,000 denier with a spinning titer of the individual filaments of 11.8 denier. The cable was treated as described in Example 5. The data and textile properties of the final product are recited in the following Table 2. A comparison with Example 5 reveals that with the dyestuff receptivity the number of spinning defects is considerably lower when the present mixture was used instead of a polyethylene terephthalate having a very low medium molecular weight.

### EXAMPLE 7

A mixture of 90 parts of polyethylene terephthalate having a specific viscosity  $\eta_{sp}$  of 0.47 and 10 parts of polyethylene terephthalate having a specific viscosity  $\eta_{sp}$  of 0.82 was melted at 260° C. in a melting device with the exclusion of air and with an extruder a wire having a diameter of 3 mm. was made. This wire was cut into 4 mm. long pieces which were fed to a melt spinning apparatus.

From the fibers a spinning cable was formed having total titer of 165,000 denier, while the individual fibers had a spinning titer of 11.7 denier. The cable was treated as described in Example 5. The data and textile properties of the cable are indicated in the following Table 2. A comparison with Examples 5 and 6 reveals that with a dyestuff receptivity of 52% the lowest number of spinning defects is obtained when 90 parts of polyethylene terephthalate having an especially low medium molecular weight are mixed with 10 parts of polyethylene terephthalate having a normal medium molecular weight, the mixture is melted and homogenized and the product obtained is then spun from the melt.

The number of defects, the agglutinations or drop-like knots in the final product were determined by taking samples.

invention have good textile and tinctorial properties and, furthermore, they have little or no tendency to pilling, this being very important in textile industries.

Table 2

| Example No.                                               | 5          | 6                    | 7                                            |
|-----------------------------------------------------------|------------|----------------------|----------------------------------------------|
| $\eta_{sp}$ of polymer                                    | 100%, 0.46 | 90%, 0.46; 10%, 0.82 | 90%, 0.47 previously; 10%, 0.82 homogenized. |
| Titer of spinning cable, denier                           | 600,000    | 150,000              | 165,000                                      |
| Spinning titer of individual filaments, denier            | 11.7       | 11.8                 | 11.7                                         |
| Conveying speeds, meters per minute:                      |            |                      |                                              |
| Prior to stretching                                       | 10.1       | 10.0                 | 10.0                                         |
| After stretching                                          | 40.4       | 41.6                 | 41.5                                         |
| After shrinkage                                           | 35.4       | 36.2                 | 36.0                                         |
| After second stretching                                   | 39.9       | 41.0                 | 41.2                                         |
| Temperature, °C.:                                         |            |                      |                                              |
| During shrinkage                                          | 234        | 233                  | 233                                          |
| During second stretching                                  | 150        | 155                  | 155                                          |
| Individual titer, denier                                  | 3.3        | 3.2                  | 3.3                                          |
| Tensile strength, g./denier                               | 2.8        | 3.0                  | 3.1                                          |
| Elongation at break, percent                              | 48         | 42                   | 46                                           |
| Shrinkage at 200 °C., percent                             | 2.4        | 7.4                  | 5.3                                          |
| Dyestuff receptivity, percent                             | 61         | 61                   | 52                                           |
| Number of spinning defects per 100 kilograms of material. | 25         | 6.8                  | 4.9                                          |

## EXAMPLE 8

A spinning cable having a total titer of 100,000 denier and a spinning titer (titer of unstretched individual filaments) of 11.7 denier of polyethylene terephthalate having a specific viscosity  $\eta_{sp}$  of 0.82 was stretched in steam, continuously allowed to shrink while being heated with contact heating and then stretched again while heated under contact. The cable was then treated with a scrooping agent, crimped and cut. The contact heating for the shrinkage after the first stretching took place on a 5 m. long vaulted surface which was heated at 245° C. and covered with a layer of glass silk (7 filaments/cm. in chain and warp, 290 grams per square meter). At a distance of 25 mm. a second heated surface which was likewise heated at 245° C. but did not touch the fiber cable was placed opposite the first one.

The conveying speeds of the individual stages and temperatures as well as the dye receptivity of the final product are given in the following Table 3. In said table the values are compared with the values of a material which had been produced in the same manner with the exception that the fiber cable directly contacted the heated metallic surface during the shrinking process. Thus, the temperature of the heating device had to be lower and the degree of shrinkage the cable underwent was likewise lower. This resulted in not so high a dyestuff receptivity of the treated fibers.

Table 3

|                                                                                | Example 8 | Comparison |
|--------------------------------------------------------------------------------|-----------|------------|
| $\eta_{sp}$ of polymer                                                         | 0.82      | 0.82       |
| Titer of spinning cable denier                                                 | 100,000   | 100,000    |
| Spinning titer of individual filaments, denier                                 | 11.7      | 11.7       |
| Conveying speeds, meters per minute:                                           |           |            |
| Prior to stretching                                                            | 10.4      | 10.0       |
| After stretching                                                               | 46.4      | 44.6       |
| After shrinkage                                                                | 35.2      | 35.5       |
| After second stretching                                                        | 38.5      | 38.7       |
| Relative shrinkage, calculated on the conveying speed after shrinkage, percent | 31        | 25         |
| Temperature of the heating surfaces, °C.:                                      |           |            |
| For the shrinkage                                                              | 245       | 215        |
| For the second stretching                                                      | 100       | 100        |
| Dyestuff receptivity, percent                                                  | 42        | 25         |

It is obvious from the above table that the application of a thin and smooth layer having poor heat-conducting properties to the heating surface involves an increase of the dyestuff receptivity from 25% to 42%, for example, without agglutinations of the fibers occurring.

The fibers and filaments treated by the process of the

We claim:

1. A process for the manufacture of filamentous structures of polyethylene terephthalate which have an improved dyeability which comprises stretching the filamentous structures to a multiple of their original length, shrinking the filamentous structures by 8 to 40% at a temperature above 190° C.; and then stretching the filamentous structures a second time by at least 3% up to at most the breaking limit of said filamentous structures.
2. A process for the manufacture of filamentous structures of polyethylene terephthalate which have an improved dyeability which comprises stretching the filamentous structures under heated conditions to a multiple of their original length, shrinking said structures by 8 to 40% at a temperature above 190° C., and stretching them a second time by at least 3% up to at most the breaking limit of said filamentous structures.
3. A process for the maintenance of filamentous structures of polyethylene terephthalate which have an improved dyeability which comprises stretching the filamentous structures to a multiple of their original length in several stages under heated conditions, shrinking said structures by 8 to 40% at a temperature above 190° C., and stretching them again by at least 3% up to at most the breaking limit of said structures.
4. The process of claim 1 wherein the structures are shrunk at 220° C.
5. The process of claim 1 wherein the filamentous structures are shrunk at a temperature above 190° C. by passing the structures in contact with a heated surface covered with a thin and smooth layer having poor heat-conducting properties.
6. The process of claim 5 wherein the layer is a glass fiber fabric.
7. The process of claim 1 wherein said filamentous structures having a specific viscosity below 0.5 are treated.
8. A process as claimed in claim 1 wherein filamentous structures are prepared from a mixture of polyethylene terephthalate having a specific viscosity of less than 0.5, and up to 20% weight polyethylene terephthalate having a specific viscosity of between 0.78 and 0.84.

## References Cited in the file of this patent

## UNITED STATES PATENTS

- 2,556,295 Pace June 12, 1951  
2,948,583 Adams et al. Aug. 19, 1960

## FOREIGN PATENTS

- 586,729 Canada Nov. 10, 1959